

July 8, 1924.

1,500,594

J. R. ROSE

GASEOUS FUEL AND PROCESS OF PRODUCING SAME

Filed Aug. 13, 1917

2 Sheets-Sheet 1



INVENTOR.

James R. Rose,  
BY  
Hull, Smith, Buck & West,  
ATTORNEYS.

July 8, 1924.

1,500,594

J. R. ROSE

GASEOUS FUEL AND PROCESS OF PRODUCING SAME

Filed Aug. 13, 1917

2 Sheets-Sheet 2



INVENTOR.

James R. Rose  
BY  
Hull, Smith, Back & West,  
ATTORNEYS.

## UNITED STATES PATENT OFFICE.

JAMES R. ROSE, OF EDGEWORTH, PENNSYLVANIA, ASSIGNOR TO CARBO-OXYGEN COMPANY, OF PITTSBURGH, PENNSYLVANIA, A CORPORATION OF DELAWARE.

## GASEOUS FUEL AND PROCESS OF PRODUCING SAME.

Application filed August 13, 1917. Serial No. 185,977.

To all whom it may concern:

Be it known that I, JAMES R. ROSE, a citizen of the United States, residing at Edgeworth, in the county of Allegheny and State of Pennsylvania, have invented a certain new and useful Improvement in Gaseous Fuel and Processes of Producing Same, of which the following is a full, clear, and exact description, reference being had to the accompanying drawings.

This invention relates to a process for the manufacture of gaseous fuel, and more particularly to a process for the production of such fuel as is particularly well adapted for the cutting and welding art, also to a new gas for use in such art. The general object of the invention is to produce a fuel which shall be more efficient than those which have been employed heretofore for this purpose and one which may contain desirable proportions of the higher and richer members of the hydrocarbon series as well as a certain amount of carbon monoxide.

Further and more generally stated, the invention may be defined as consisting of the combinations of steps embodied in the claims hereto attached and forming part hereof.

The process is conveniently realized in and through the apparatus illustrated in the drawings, wherein Fig. 1 represents a longitudinal vertical sectional view through such apparatus; Fig. 2 a view, partly in section and partly in plan, of the apparatus shown in Fig. 1, the section being taken just below the chamber 5 of the generator; and Fig. 3 a detail in elevation of one of the pieces of refractory material within the generator.

Describing by reference characters the various parts illustrated herein, 1 denotes the outer shell and 2 the refractory lining of a generator, the generator being shown as cylindrical. This refractory lining may be of any suitable well-known material, and the generator is so constructed as to provide a front flue 3 and a rear flue 4 communicating at their upper ends by a transverse passageway 5, said passageway being formed within the said lining and filler. Refractory porous material 2<sup>a</sup> is arranged in "checker-work" formation within the flues 3 and 4.

It will be observed that the bottoms of the flues 3 and 4 are located at a distance above the bottom of the generator body, whereby

ample thickness of refractory material 2<sup>b</sup> is provided below such flues.

6 denotes a partition, preferably of sheet steel, extending transversely across the generator between the flues 3 and 4 and extending from the bottom of the generator upwardly to a distance below the top of the refractory dividing wall 2<sup>c</sup>. This partition prevents seepage of gases from the flue on one side thereof to the flue on the opposite side thereof. 7 denotes an inlet connection 65 communicating with the front or charging wall of the generator and discharging into the bottom of the flue 3. This connection is provided at its outer end with a gate valve 8 and is extended, as indicated at 9, to a suitable air blower (not shown). 10 denotes a nozzle through which a suitable preheating fluid (such as hydrogen, or natural gas, or a mixture of the same) mixed with air (supplied through the connection 9) may be introduced into the bottom of the flue 3 beneath the arch 3<sup>b</sup>. This nozzle preferably extends axially into the connection 7 and is adapted to receive the gaseous fuel from the pipes 11 and 11<sup>a</sup>, respectively, each of said pipes having a valve, indicated at 11<sup>b</sup> and 11<sup>c</sup> respectively. Hydrogen may be supplied by the pipe 11, and natural gas through the pipe 11<sup>a</sup>. The hydrogen and natural gas are admitted separately to form the mixture 75 to be treated.

The flues 3 and 4 are provided each with a checker-work filling of porous refractory material, referred to hereinbefore and indicated at 2<sup>a</sup>, while the transverse flue 5 is provided with an outlet connection 12 having a weighted blow-off or pressure-relief valve therein, the operating handle whereof is indicated at 13. From the arch 4<sup>a</sup> at the bottom of the flue 4, there extends an outlet 80 flue 14 the discharge end of which projects into a receptacle 15, the lower end 14<sup>a</sup> of such flue being sealed by suitable liquid within the said receptacle. Projecting upwardly from the outlet flue 14 is a pipe 16 85 having a pressure-relief valve therein similar to the valve in the pipe 12, the operating handle of the valve being indicated at 17.

From the top of the receptacle 15, and having its inlet end above the liquid therein, 90 extends a pipe 18 which communicates with the bottom of the scrubbing tank 19, having a series of transverse, perforated partitions

20 therein with suitable porous material 21, such as pumice stone, on said partitions and a spraying nozzle 22 in the upper end thereof of above the uppermost partition and the 5 material thereon. From this scrubber a pipe 23 extends into a tank 24 which may contain a hydrocarbon liquid of one of the higher or richer series, the pipe 23 being provided with perforations 23<sup>a</sup> beneath the top of the 10 liquid in said tank whereby the gas discharged from the scrubber may be further enriched. From the enriching tank 24 a pipe 25 leads to a storage tank or to the point of use. From the front of the furnace 15 1, there project pipes or connections 26 which provide means for applying pyrometers to the flue 3 or for the application of instruments for estimating the temperature by observation, as by a color test. In operation, 20 the hydrogen or natural gas or a mixture of the same, will be introduced into the bottom of the flue 3 from the pipes 11 and 11<sup>a</sup>, together with an excess of air admitted through the connections 7 and 9. This mixture, 25 being ignited, burns in contact with the refractory material 2<sup>a</sup> in the flues 3 and 4 until the desired temperature (not materially lower than 1600° F.) is attained, as indicated by the pyrometers or sight tubes. 30 The products of combustion resulting from this preheating operation will escape through the upper end of the pipe 16, the valve being opened or lifted by its handle 17 for the purpose of facilitating the discharge of such gases.

After the "blowing-up" or preheating operation, hydrogen and natural gas are supplied to the generator and are there subjected to a temperature not materially lower 40 than 1600° F. The temperature will be sufficient to dissociate the natural gas into carbon and hydrogen in a nascent condition, and a recombination will be effected whereby the resultant fixed gas discharged from 45 the generator will contain a higher proportion of hydrogen and a lower percentage of methane than were supplied through the connection 7, together with free carbon and a small proportion of carbon monoxide. In 50 general, the higher the temperature, the higher will be the proportion of the hydrogen and the lower the proportion of the methane constituent of the resultant gas. At a temperature of 2200° F. the gas discharged 55 from the generator will contain about 85 per cent of hydrogen and from 13 to 14 per cent of methane, together with from 1 to 2 per cent of carbon monoxide, which is produced by the combination of some of the 60 carbon constituent of the dissociated natural gas with oxygen occluded within the pores of the refractory material from the preheating operation, the oxygen being taken from the excess air supplied with the gaseous 65 fuel during the preheating operation. If the

temperature of the generator is lower than 2200° F., the proportion of hydrogen in the final gas will be lower and the proportion of methane higher than at such temperature; on the other hand, if the temperature to 70 which the gases are subjected be increased, the proportion of methane will be diminished and the proportion of hydrogen increased. The resultant gas, however, will contain hydrogen, methane, and carbon 75 monoxide, and will be fixed and permanent at a temperature of at least 100° below zero F., and under a pressure of 1800 pounds.

The gas which has been produced within the generator is conducted through the receptacle 15, which will trap the solid carbon produced by the dissociation of the natural gas; thence the gas may be conducted through the scrubbing tank 19 and thence to the enriching tank 24.

The hydrocarbon liquid in the tank 24 may be benzene, naphthalene, or any other volatile hydrocarbon of a sufficiently high series, and the resultant fluid will not separate or stratify when stored under pressure.

It is to be observed that, by the dissociation of the natural gas in the presence of the refractory material, the resultant fixed gas contains hydrogen and methane in different proportions from those in which hydrogen and natural gas were supplied to said material and that the resultant gas contains in addition a small but valuable proportion of carbon monoxide. The carbon, in the form of lamp black may be recovered 100 from the receptacle 15.

Having thus described my invention, what I claim is:

1. The process of producing gaseous fuel which comprises subjecting a mixture of hydrogen and natural gas to a temperature sufficient to dissociate the natural gas, and subjecting the resultant mixture to a temperature not materially lower than 1600° F. in the presence of oxygen.

2. The process of producing gaseous fuel which comprises subjecting a mixture of hydrogen and natural gas admitted separately to a chamber containing porous refractory material heated to a temperature not materially lower than 1600° F.

3. The process of producing gaseous fuel which comprises heating refractory porous material by means of gases burning in an excess of oxygen thereby to raise the temperature of such material to a point not materially lower than 1600° F. and to occlude oxygen in the pores of such material, and subjecting a mixture of hydrogen and natural gas to the action of such heated material.

4. The process of producing gaseous fuel which comprises subjecting a mixture of hydrogen and natural gas to the action of porous refractory material containing oxy-

gen in the pores thereof and heated to a temperature not materially lower than 1600° F., and removing from the resultant gas free 10 carbon caused by the dissociation of the natural gas.

5. The process of producing gaseous fuel which comprises subjecting a mixture of hydrogen and natural gas to the action of porous refractory material containing oxygen in the pores thereof and heated to a tem-

perature not materially lower than 1600° F., and removing from the resultant gas free 10 carbon caused by the dissociation of the natural gas.

In testimony whereof, I hereunto affix my signature.

JAMES R. ROSE.